# EUROPEAN PATENT APPLICATION

(11) **EP 4 786 663 A1**
(43) Date of publication of application: **05.08.2026**
(21) Application number: 26153554.6
(22) Date of filing: 22.01.2026
(51) Int. Cl.: D03D 15/41, D03D 15/43, D03D 27/08, D02G 3/28, D03D 15/217

(54) **A SOFT TWIST TERRY FABRIC AND A METHOD OF MANUFACTURING THEREOF**

(30) Priority: 29.12.2025 IN 202511133227
(71) Applicant: Trident Limited, 148101 Pumjab (IN)
(72) Inventor: Gupta, Abhishek, 141001 Ludhiana (IN)
(74) Representative: Potter Clarkson

(57) **Abstract**

The present invention discloses a soft twist terry fabric and a manufacturing method thereof that produces upright, profiled pile loops with high bulk, softness, and durable loop stability without zero-twist constructions or water-soluble fibers or other conventional techniques that compromise loop stability and environmental sustainability. Each pile loop is formed from a plied pile yarn comprising a coarse yarn and a fine yarn twisted in opposite directions and plied by Two-For-One twisting in the fine yarn's direction. Controlled plying operation is employed to yield a balloon-like spiral cover at the loop crown and a spring-like fine yarn at the loop base. A fine-yarn helical wrap angle of about 15°-30° is obtained relative to the plied yarn axis and at least two fine-yarn turns per loop is obtained for root firmness and shape retention. The process further stabilizes spirality and reduces linting by approximately 20-40% after repeated washes.

## Description

### Field of the invention

The present invention relates generally to the field of manufacturing soft terry fabrics. More particularly, the present invention relates to a soft twist terry fabric that exhibits enhanced bulkiness and softness, reduced shedding and loop retention, and a controlled and environment friendly manufacturing process thereof.

### Background of the invention

Terry fabrics are a class of pile fabrics produced by weaving or related fabric-forming processes in which additional yarns are introduced to form loops (also referred to as pile loops) on one or both surfaces of a woven base. Terry fabrics are commonly used in towels, bathrobes, rugs, bath mats, and similar absorbent articles. Properties and performance of terry fabrics are based on multiple design and process parameters including fiber type, yarn count and construction, pile height and density, ground weave, and overall fabric weight. End users of terry fabrics typically seek high softness, superior moisture absorbency, and a uniform, visually appealing surface with durable loop formation.

Conventional approaches to achieving soft terry fabrics include the use of "zero twist," "low twist," and "air-rich" yarns. In many such techniques, a water-soluble fiber, for example polyvinyl alcohol (PVA) is employed to create voids or to facilitate twist removal prior to weaving. Although these methods can produce a soft hand feel, they are associated with significant drawbacks. PVA contributes to yield loss, involves energy intensive processing and creates non-biodegradable effluents which raises environmental and waste management concerns as it precipitates and affects downstream treatment. Also, PVA and similar soluble components have relatively low strength and high elongation which complicates weaving and process stability.

Furthermore, typically, terry fabrics made with low twist or zero twist yarns exhibit functional and aesthetic shortcomings during use and care. Cottons portion of zero-twist constructions often exhibit reduced strength. Also, loop configuration of these yarns tends to bend or compress due to yarn softness and insufficient structural integrity which lead to reduced apparent bulk for a given pile height. Loose fibers readily detach from the loops during washing which causes linting, fuzz formation, and hairiness, that degrade appearance and hand feel over time. The surface of such fabrics can appear irregular or uneven after laundering. Illustrative images of prior art terry fabrics in which bent loops, fuzz, and surface irregularity are observed are shown in Figs. 1A-1B. Even where PVA is avoided, some low-twist or composite-yarn constructions exhibit higher lint loss and surface instability after multiple washes. In many cases, loop geometry degrades over time which compromises absorbency, bulk, and hand feel. These issues are accompanied by process complexity and the sensitivity of pile formation to twist levels, twist direction combinations, and finishing conditions, which often lead to inconsistent results across production batches.

Other known methods attempt to produce softness using combinations of thick and thin yarns, often through Two-for-One (TFO) twisting and related doubling practices. However, when thick and thin yarns are twisted in the same direction without adequate control of twist interactions, pile loops can lack a well-defined upright structure and fail to deliver the desired combination of softness, bulk, and stability. Uncontrolled migration and spirality of constituent yarn plies yield inconsistent internal structure, leading to loop instability, surface non-uniformity, and variability in pile inclination and retention. As a result, the perceived bulk in the final product may be lower than the nominal pile height, and the loops may not remain sufficiently upright to maintain a plush profile. Representative images showing inadequate loop formation and surface irregularities in prior art fabrics are illustrated in Figs. 1A-1B.

Yet further, pile profile which includes parameters such as pile inclination angle and loop firmness materially affect perceived bulk and softness. In existing soft constructions using low or zero twist yarns, the pile inclination angle tends to be relatively low and loops are prone to bending, thereby diminishing the apparent thickness for a given loop length. Conversely, in other constructions where higher pile inclination is achieved, loops made with soft one-ply or two-ply yarns may still lack the desired softness or loop definition and can present uneven surfaces and hairiness after use and washing, as shown in exemplary images of prior art in Figs. 1A-1B.

In light of the aforementioned drawbacks, there is a need for a method for manufacturing terry fabrics that exhibit a high pile profile with increased softness and firm loops. There is a need for manufacturing terry fabrics having upright loop configuration that resists bending, delivers durable bulk, and maintains a regular, uniform surface over repeated washes. There is also a need to manufacture terry fabrics that exhibit reduced linting and fiber shredding while improving absorbency and tactile properties, without relying on water-soluble synthetic fibers that cause yield loss and environmental concerns. Further, there is a need for manufacturing terry fabrics that provide consistent loop geometry and pile orientation, improved pile stability and surface integrity, and that are cost-effective, scalable, and environmentally favorable.

### Summary of the Invention

A soft twist terry fabric is provided in accordance with an embodiment of the present invention. The soft twist terry fabric comprises a woven ground fabric of warp and weft yarns and a plurality of upright profiled pile loops formed on one or both surfaces of the fabric. Each pile loop comprises a plied pile yarn constructed from a coarse yarn twisted in a first direction and a fine yarn twisted in a second direction opposite to the first twist direction and the coarse and fine yarns are doubled and plied using a Two-for-One (TFO) twisting technique in the fine yarn's twist direction to form a fine yarn wrap. The warp yarns, weft yarns, coarse yarns, and fine yarns are made from fibers selected from natural fibers, synthetic fibers, blended fibers, regenerative fibers or any combination thereof. The structure of each of the pile loops formed is such that the coarse yarn forms a ballon-like spiral cover within a crown region of each of the pile loops. The spiral cover is induced by partial opening of the coarse yarn structure under the opposite-direction fine yarn wrap, thereby imparting enhanced softness, bulk, and reduced fiber protrusion. The fine yarn is positioned predominantly towards a base of each of the pile loops, acting as a spring element to provide radial confinement and base support. The plied pile yarn exhibits a helical wrap angle of the fine yarn in a range from 15 degree to 30 degrees relative to the plied yarn axis. The structure of the pile loops is achieved by controlling the plying process such that the fine yarn contributes at least two turns per terry loop which ensures loop stability and shape retention. The soft twist terry fabric provides enhanced bulk, improved hand feel, reduced shedding or loose fibers and lint release during use and laundering, and durable uprightness of pile loops after repeated washes.

A method of manufacturing a soft twist terry fabric is provided in accordance with an embodiment of the present invention. The method comprises providing a coarse yarn and a fine yarn made from fibers selected from natural fibers, synthetic fibers, blended fibers, regenerative fibers, or any combination thereof. The coarse yarn is twisted in a first twist direction and the fine yarn is twisted in a second twist direction opposite to the first twist direction. The twist multipliers of the coarse yarn and the fine yarn are preset within predetermined ranges suitable for pile yarn formation prior to plying. The fine yarn is wrapped around the coarse yarn by further twisting the fine yarn in said second direction to form a helical, balloon-like spiral wrap that partially opens the twisted structure of the coarse yarn along its length. The coarse yarn and the fine yarn are plied using a Two-For-One (TFO) twisting technique under controlled tension and twist insertion to obtain a plied pile yarn, wherein the plying operation is controlled such that, upon fabric formation, the fine yarn contributes at least two turns per terry loop and the fine yarn migrates towards a base of each of the pile loops to provide a radial confinement and base support while the coarse yarn occupies the loop crown region to maximize an opening volume within the loop structure, thereby producing a plied pile yarn in which the coarse yarn remains structurally bulked and the fine yarn acts as a confinement wrap. The plied pile is woven into a terry fabric to form upright profiled pile loops, whereby the terry fabric exhibits enhanced bulk and improved hand feel, and the plied pile yarn exhibits reduced shedding of loose fibers after weaving relative to a comparable terry fabric produced without the opposite-direction fine-yarn wrapping and TFO-controlled loop architecture.

### Brief description of the accompanying drawings

The present invention is described by way of embodiments illustrated in the accompanying drawings wherein:
Figs. 1A and1B represent images of prior art terry fabrics;
Fig. 1C shows an image of the soft twist terry fabric (towel) manufactured in accordance with an embodiment of the present invention;
Fig. 2 illustrates a cross-sectional view of a soft twist terry fabric, in accordance with an embodiment of the present invention;
FIG. 3 illustrates a cross-sectional view of a plied pile yarn with a profiled pile loop having a defined helical wrap angle and two turns of fine yarn per loop, in accordance with an embodiment of the present invention; and
FIG. 4 illustrates a helical wrap angle made by the fine yarn relative to the plied pile yarn axis, in accordance with an embodiment of the present invention.

### Detailed description of the invention

In various embodiments of the present invention, a method for manufacturing soft twist terry fabrics is provided. The present invention discloses making a soft twist terry fabric with upright, profiled loops with durable bulk, softness, and reduced linting without relying on zero-twist constructions or soluble fibers or other conventional techniques that compromise loop stability and environmental sustainability. The soft twist terry fabric of the present invention exhibits a high pile profile with a firm upright loop configuration that resists bending, delivers durable bulk, and maintains a regular, uniform surface over repeated washes. The soft twist terry fabric of the present invention exhibits reduced linting and fiber shredding while improving absorbency and tactile properties, without relying on water-soluble synthetic fibers that cause yield loss and environmental concerns. Further, the manufacturing process of the present invention produces the soft twist terry fabric with consistent loop geometry and pile orientation, improved pile stability and surface integrity, and that are cost-effective, scalable, and environmentally favorable.

The disclosure is provided in order to enable a person having ordinary skill in the art to practice the invention. Exemplary embodiments herein are provided only for illustrative purposes and various modifications will be readily apparent to a person skilled in the art. The general principles defined herein may be applied to other embodiments and applications without departing from the scope of the invention. The terminology and phraseology used herein is for the purpose of describing exemplary embodiments and should not be considered limiting. Thus, the present invention is to be accorded the widest scope encompassing numerous alternatives, modifications, and equivalents consistent with the principles and features disclosed herein. For purposes of clarity, details relating to technical material that is known in the technical fields related to the invention have been briefly described or omitted so as not to unnecessarily obscure the present invention.

The present invention would now be discussed in context of embodiments as illustrated in the accompanying drawings.

Fig. 1C illustrates a soft twist terry fabric, according to an embodiment of the present invention. In this figure, the soft twist terry fabric demonstrated is a towel. As illustrated in Fig. 1C, the loop structure of the soft twist terry fabric comprises of a profiled pile loop which are substantially upright, well-rounded, and consistently formed, thereby providing a stable, well-supported pile with a pronounced plush profile. The soft twist terry fabric, made in accordance with the present invention, demonstrates an elevated bulk, a soft hand feel, and high absorbency with a smooth and even surface that is substantially free from fuzz and hairiness. The loops retain their shape without appreciable tilting or collapse, thereby yielding a uniform appearance and tactile consistency across the fabric plane. Compared with representative prior art examples shown in Figs. 1A-1B, the soft twist fabric shows reduced linting, reduced fuzz formation during laundering and improved surface regularity. Moreover, the bulk, softness, absorbency, and surface cleanliness of the soft twist terry fabric are maintained after multiple wash cycles which indicates durable uprightness (loop stability) and a long-lasting quality in a soft terry fabric.

Fig. 2 depicts a cross-sectional view of the soft twist terry fabric, in accordance with an embodiment of the present invention. In this embodiment of the present invention, a two-ply or a multi-ply yarn construction is employed to produce the terry fabric by weaving warp 207 and weft 208 yarns with a plurality of plied pile yarns to form the pile loops 202 formed on one or both surfaces of the resulting terry fabric. Within each loop 202, the yarns separate out into distinct positions as indicated by reference numerals 204 and 206 for a coarse and a fine yarn respectively. This loop structure provides a robust surface profile with enhanced firmness and roundness of the loops formed on the terry fabric. The loop structure shown in Fig. 2 yields excellent surface integrity characterized by low hairiness, uniform loop occurrence and distribution, and an absence of noticeable defects throughout the cross-section of the finished soft twist terry fabric.

In this embodiment of the present invention, the profiled loop configuration of the resultant soft twist terry fabric is obtained through a manufacturing method comprising a controlled soft twist process using two-ply yarns or multi-ply yarns. In this method, firstly, two yarns are provided which are a relatively coarse or thick yarn and a relatively fine yarn. The counts of the coarse and fine yarns are chosen in accordance with the targeted fabric Grams per square meter (GSM), cover factor, and pile height such that the coarse yarn provides a spiral cover while the fine yarn contributes anchoring and resilience at the loop base. In an example, the coarse or thick yarn having yarn count in a range from 6 Ne to 30 Ne and a fine yarn having yarn count in a range from 20 Ne to 177 Ne are selected. In another example, the warp yarns, weft yarns, coarse yarns, and fine yarns are made from fibers selected from natural fibers, synthetic fibers, blended fibers, regenerative fibers, or any combination thereof. In another example, the coarse, fine yarn, warp yarn and weft yarn are independently selected from fibers comprising Organic cotton, BCI cotton, Indian cotton, USA cotton, Supima cotton, Egyptian cotton, Australian cotton, Turkish cotton, naturally colored cotton, naturally dyed cotton, dyed cotton, cotton blended with regenerated or synthetic fibers, cotton/bamboo, cotton/modal, cotton/micro-modal, cotton/tencel, cotton/viscose, cotton/silk, cotton/bamboo/hemp, cotton/hemp, cotton/linen, cotton/ecover, cotton/excel, Egyptian cotton/excel, recycled cotton and its blends, cotton/Naia, cotton/wool, cotton/PVA, cotton/polyester, Regenerative cotton, Kasturi cotton, cotton/PLA, or any combination thereof. In another exemplary embodiment of the present invention, the fine coarse yarn and the fine yarn can be woven using a 2 pick, 3 pick or 4 pick weaving technique.

Secondly, the coarse single yarn is twisted in a first twist direction , either clockwise or counterclockwise direction, and the fine single yarn is twisted in a second twist direction opposite to the first twist direction of the coarse yarn. For example, if the direction of the twist applied to the coarse single yarn is in the clockwise direction, then the fine yarn is twisted in the counterclockwise direction, and vice versa. The Twist Multipliers (TM) of the single yarns are preset within predetermined ranges prior to plying the coarse and thin yarns. TM in textiles is a calculated factor that relates yarn's twist level (turns per inch/meter) to its thickness (yarn count) which determines the ideal twist for strength. In this embodiment of the present invention, the formula used is TM = TPI / √Yarn Count which indicates how much twist is needed for different yarn sizes to achieve a consistent yarn. In an example, the coarse yarn is prepared with a TM in a range from 2.6-3.8 and the fine yarn is prepared with a TM in a range from 3.0-4.8. In this embodiment of the present invention, fine yarn is wrapped around the coarse yarn in the said second direction to form a helical, balloon-like spiral wrap that partially opens the twisted structure of the coarse yarn along its length, which results in producing a plied yarn in which the coarse yarn remains structurally bulked and the fine yarn acts as a confinement wrap after a plying operation is carried out.

Thirdly, the plying operation is carried out to produce a plied pile yarn. The coarse single yarn within the specified range of TM and twisted in the first direction (clockwise or counterclockwise), and the fine single yarn within the specified range of TM and twisted in the second direction opposite to the twisting direction of the coarse single yarn are doubled and plied under controlled tension and twist insertion in the twisting direction of the fine single yarn using a Two-For-One (TFO) twisting technique to produce a plied pile yarn as schematically depicted in Fig. 3. In this embodiment of the present invention, the plying tension applied to the fine yarn is greater than plying tension applied to the coarse yarn, thereby biasing migration of the fine yarn toward the loop base. The plying operation is controlled to yield a defined plied helical wrap angle in a range from 15°-30° relative to the plied yarn axis. The helical wrap angle in plied yarn loops, such as in a rope or fabric, is the angle that an individual fiber strand or yarn makes with a longitudinal axis of the entire plied structure. The helical wrap angle is the angle that the fine yarn makes with the longitudinal axis of the plied pile yarn produced after the plying operation, as illustrated in Fig. 4. In an example, the helical wrap angle is measured by the formula tan(θ) = (π× D × TPI), wherein, θ = Helical wrap angle, D= yarn diameter inches, TPI = Twists per Inch of fine yarn.

In this embodiment of the present invention, the plying of the single yarns to produce the plied pile yarn is carried out by ensuring at least two turns of fine-yarn per terry loop. Two turns of fine yarn per loop are ensured by pre-setting the TPI of the plied pile yarn such that in the plied pile loop geometry the fine yarn contributes at least two turns per loop. TPI is a measurement of how many times the yarn fibers are twisted around their own axis within a one-inch length. TPI is selected within a pre-defined range based on a target pile height. For example, TPI is selected within a range from 2.5-13.5 for a target pile height of about 2.5-10 mm, so that shorter piles employ higher TPI and taller piles employ mid-range TPI while consistently maintaining the fine-yarn turns-per-loop threshold. The fine yarn is wrapped around each individual pile loop with at least two turns, thereby providing maximum opening space for the coarse yarn within the loop structure to enhance bulk and improve hand feel.

In this embodiment of the present invention, the plying operation is carried out via a controlled process wherein parameters associated with the individual yarns and the plying operation are preset. The preset parameters of the single yarns like the TM and yarn count ensure that upon weaving into a terry fabric, the coarse component of the plied pile yarn presents a low-to-moderate resultant twist. Therefore, the coarse component is extended away from the base of the fabric and results in overfeeding which promotes softness and bulk. Whereas, the fine component of the plied yarn presents a relatively higher effective twist that anchors at the loop base and resists loop bending under pressure during use and laundering. This ensures that fine yarn migrates towards the base of the loop and acts as a spring to provide radial confinement and base support while the coarse yarn wraps helically as a spiral cover. The coarse yarn occupies the loop crown region to maximize an opening volume within the loop structure, thereby producing a plied pile yarn in which the coarse yarn remains structurally bulked and fine yarn acts as a confinement wrap. The pre-setting of individual-yarn TM ranges also enables achieving the helical wrap-angle and turns-per-loop targets without resorting to excessive plying twist that would otherwise stiffen the fabric or destabilize the loops. The TMs of the fine coarse and fine yarn are selected to permit partial opening of the coarse yarn under the fine yarn wrap without collapse of the coarse yarn during plying. Also, ensuring at least two fine-yarn turns per loop at the selected helical wrap angle results in the loop structure of the spiral soft twist terry fabric to have improved root firmness, loop stability, shape retention, and surface integrity over time.

Through multiple experimentations, it has been ascertained that if the fine yarn contributes fewer than two turns per loop, anchoring at the loop root is insufficient and loops tend to bend. The 15°-30° window for the helical wrap angle is selected to provide sufficient radial confinement and base support without over-compressing the loop structure, thereby preserving porosity and hand feel of the spiral soft twist terry fabric while stabilizing loop uprightness. It has been observed that a helical wrap angle below 150° produces a shallow spiral with weak radial compression, leading to poor loop-base support and higher lint under pressure or wear and tear, whereas a helical wrap angle above about 30° induces excessive radial compression that reduces porosity and capillarity, hardens hand feel, and can trigger torque instabilities. It has been observed that if TPI is driven excessively high, openness and softness may be restricted and loop torque may increase. As a result, the plied pile yarn of the soft twist terry fabric exhibits a controlled spirality in which the coarse component acts as a spiral cover while the fine component stores sufficient spring energy to reinforce the loop root. In this embodiment of the present invention, the helical spiral wrap of the fine yarn forms a continuous wrap along the coarse yarn with a pitch selected to maintain radial confinement at the loop base region during terry weaving.

Working Examples: Working examples for obtaining the helical angle range from 15 to 30 degrees by using the preset values of the parameters are shown below:
Example1 - If a coarse count has 10 Ne and fine count having 30 Ne and twisting at TFO around 13.5 TPI
   Component Count- 10 Ne &30 Ne
   Resultant Count- 7.50 Ne
   Calculated Diameter- 0.01312 inch
   tan(θ)- 0.268
   Helical wrap angle - 15 degree
Example2 - If a coarse count has 10 Ne and fine count having 60 Ne and twisting at TFO around 10.5 TPI
   Component Count- 10Ne & 60 Ne
   Resultant Count- 8.57 Ne
   Calculated Dia- 0.0122 inch
   tan(θ)- 0.402
   Helical wrap angle - 22 degree
Example3 - If a coarse count has 10 Ne and fine count having 80 Ne and twisting at TFO around 8.5 TPI
   Component Count- 10Ne & 80 Ne
   Resultant Count- 8.89 Ne
   Calculated Dia- 0.0120 inch
   tan(θ)- 0.32
   Helical wrap angle - 18 degree
Example4 - If a coarse count has 9 Ne and fine count having 30 Ne and twisting at TFO around 6.5 TPI
   Component Count- 09 Ne &30 Ne
   Resultant Count- 6.92 Ne
   Calculated Dia- 0.0136 inch
   tan(θ)- 0.577
   Helical wrap angle - 30 degree

In an example, the individual-yarn TMs in the range of 2.6-3.8 for the coarse single yarn and 3.0-4.8 for the fine single yarn, a controlled plied helical wrap angle of about 15°-30°, and plied TPI in the range of 2.5-13.5 results in at least two fine-yarn turns per loop across pile heights of about 2.5-10 mm, which yields profiled pile loops that remain upright, rounded, and consistent, with high compressibility and recovery in the soft twist terry fabric. Advantageously, fabrics manufactured in accordance with these embodiments exhibit high bulk and softness with loop firmness which results in enhanced absorbency as compared to conventional soft terry fabrics at similar specifications, and a reduction in lint release in the order of about 20-40% relative to conventional constructions. The soft twist terry fabric also maintains a uniform, fuzz-free surface after multiple wash cycles. Loop retention of the soft twist terry fabric over laundering is a result of the balanced torsional "spring" of the fine yarn within the 15°-30° helical wrap angle window and the anchoring effect of the threshold based fine turns per loop topology.

In this embodiment of the present invention, the soft twist terry fabric is produced by weaving warp 207 and weft 208 yarns to form a woven ground fabric of warp and weft yarns, with a plurality of upright pile loops 202 formed on one or both surfaces of the resulting fabric, wherein the terry fabric exhibits enhanced bulk and improved hand feel, and the plied pile yarn exhibits reduced shedding of loose fibers after weaving relative to a comparable terry fabric produced without the opposite-direction fine-yarn wrapping and TFO-controlled loop structure. In an embodiment of the present invention, the warp yarns 207, weft yarns 208, coarse yarn 204 and fine yarn 206 are woven from a plurality of fiber types, as mentioned above. The plied pile yarn is woven on a terry loom to yield the profiled pile loops having a loop height and density selected to preserve the partial opening of the coarse yarn crown region.

In this embodiment of the present invention, following weaving, the terry fabric is subjected to a two-sided, to-and-fro tumbling process on a tumbling machine with optimized tumbling parameters to stabilize loop geometry, enhance bulk and reduce linting. The bi-directional, two-and-fro tumbling process stabilizes the spiral loop geometry, opens the pile loops without compromising the loop base, and further settles the fine yarn toward the loop root, thereby mitigating twist liveliness and torque-related instabilities. This finishing step enhances bulk and handfeel in the soft twist terry fabric while reducing surface hairiness and lint release and contributes to the uniform, upright loop profile observed in the finished soft twist terry fabric. The tumbling parameters are tuned to stabilize spirality, to promote loop openness while maintaining base firmness, and to minimize residual torque so that loop inclination and surface uniformity are retained over repeated wash and use cycles. In an exemplary embodiment of the present invention, the optimized tumbling parameters are illustrated in Table 1.

**Table 1: Optimized Tumbling Parameters**

| Parameter | Value |
|---|---|
| Speed | 10-13 mpm |
| Tumbling time | 5 minutes per tumbling chamber |
| Temperature | 160-170°C |
| Fan blower | 100% |
| Finishing Recipe | Silicon & cationic agents, optionally including value-added topical finishes |
| Tumbling action & fabric | Double-side tumbling process (TTO & TTM) |

As a result of the manufacturing process in accordance with various embodiments of the present invention, the resultant terry fabric exhibits a distinctive loop structure (pile loop 202) as seen in Fig. 2 and Fig.3. Within each loop 202, the two constituent yarns remain separated into distinct positions, with the relatively coarse yarn 204 providing a balloon like helical spiral cover within the crown region of each of the pile loops and the relatively fine yarn positioned predominantly towards the loop base acting as a spring element, thereby providing radial confinement and base support. The spiral configuration of the coarse yarn is induced by the partial opening of the coarse yarn structure under the opposite direction fine yarn wrap. The coarse yarn 204, prepared within its preset single-yarn TM range, exhibits low to moderate resultant twist and higher overfeeding structure, thereby allowing fiber extension sufficient to expand and adopt a desirable ballon-like spiral shape without being harsh which contributes to enhanced bulk, softness and reduced fiber protrusion. The fine yarn 206, set by reverse twisting at TFO and finished via two-sided (to-and-fro) tumbling, retains spring-like torsional energy while avoiding uncontrolled radial compression, which stabilizes the loop at its base that causes the pile loop 202 to resist bending and collapse under pressure during use and washing. The plied pile yarn of the soft twist terry fabric exhibits a controlled helical wrap angle in the range of 15°-30° relative to the plied yarn axis, which enables the loop to remain round and maintain a well-supported profile. The structure of the pile loops is achieved by the controlled plying process such that the fine yarn contributed at least two turns per terry loop, thereby ensuring loop stability and shape retention. The TPI are selected so that the fine yarn 206 contributes at least two turns per loop which ensures stable base anchoring and consistent loop shape. The soft twist terry fabric exhibits enhanced bulk, improved hand feel, reduced shedding of loose fibers and lint release during use and laundering, and durable uprightness of pile loops after repeated washes. In accordance with various embodiments of the present invention, the per-loop topology together with the controlled helical wrap angle results in a uniform, upright loop with reduced hairiness and visible surface regularity. Further, it has been observed that the pile loops formed in accordance with the embodiments of the present invention provide for a high inclination angle in respect to the pile layer, therefore the loops formed are distinctively upright.

Advantageously, as mentioned previously, the controlled soft twist process based manufacturing comprising preset individual-yarn TM ranges, a plied helical wrap angle of about 15°-30°, and TPI selected to ensure at least two fine-yarn turns per loop is formed with the two-sided tumbling process provides an unexpectedly high bulk and softness with stable, upright loops and approximately 20-40% lower linting relative to conventional soft-twist terry.

While the exemplary embodiments of the present invention are described and illustrated herein, it will be appreciated that they are merely illustrative. It will be understood by those skilled in the art that modifications in form and detail may be made without departing from or offending the spirit and the invention.

## Claims

1. A soft twist terry fabric comprising:
a woven ground fabric of warp and weft yarns;
a plurality of upright profiled pile loops formed on one or both surfaces of the fabric, each pile loop comprising a plied pile yarn constructed from:
a coarse yarn twisted in a first twist direction; and
a fine yarn twisted in a second twist direction opposite to the first twist direction, wherein the coarse and fine yarns are doubled and plied using a Two-For-One (TFO) twisting technique in the fine yarn's twist direction to form a fine yarn wrap;
wherein the warp yarns, weft yarns, coarse yarns, and fine yarns are made from fibers selected from natural fibers, synthetic fibers, blended fibers, regenerative fibers, or any combination thereof;
wherein structure of each of the pile loops is **characterized by**:
the coarse yarn forming a balloon-like spiral cover within a crown region of each of the pile loops, said spiral cover is induced by partial opening of the coarse yarn structure under the opposite-direction fine yarn wrap, thereby imparting enhanced softness, bulk, and reduced fiber protrusion;
the fine yarn positioned predominantly towards a base of each of the pile loops base, acting as a spring element to provide radial confinement and base support;
the plied pile yarn exhibiting a helical wrap angle of the fine yarn in a range from 15° to 30° relative to the plied yarn axis; and
the structure of the pile loops being achieved by a controlled plying process such that the fine yarn contributes at least two turns per terry loop, thereby ensuring loop stability and shape retention;
wherein the soft-twist terry fabric exhibits enhanced bulk, improved hand feel, reduced shedding of loose fibers and lint release during use and laundering, and durable uprightness of pile loops after repeated washes.

2. The soft twist terry fabric as claimed in claim 1, wherein the coarse and fine yarns are independently selected from fibers comprising organic cotton, BCI cotton, Indian cotton, USA cotton, Supima cotton, Egyptian cotton, Australian cotton, Turkish cotton, naturally colored cotton, naturally dyed cotton, dyed cotton, cotton blended with regenerated or synthetic fibers, cotton/bamboo, cotton/modal, cotton/micro-modal, cotton/tencel, cotton/viscose, cotton/silk, cotton/bamboo/hemp, cotton/hemp, cotton/linen, cotton/ecover, cotton/excel, Egyptian cotton/excel, recycled cotton and its blends, cotton/Naia, cotton/wool, cotton/PVA, cotton/polyester, Regenerative cotton, Kasturi cotton, cotton/PLA, or any combination thereof;

3. The soft twist terry fabric as claimed in claim 1, wherein the fine yarn is wrapped around each individual pile loop with at least two turns, thereby providing maximum opening space for the coarse yarn within the loop structure to enhance bulk and improve hand feel.

4. A method for manufacturing a soft twist terry fabric, the method comprising:
providing a coarse yarn and a fine yarn made from fibers selected from natural fibers, synthetic fibers, blended fibers, regenerative fibers, or any combination thereof;
twisting the coarse yarn in a first twist direction and the fine yarn in a second twist direction opposite to the first twist direction, wherein Twist Multipliers (TM) of the coarse yarn and the fine yarn are preset within predetermined ranges suitable for pile yarn formation prior to plying; **characterized by**
wrapping the fine yarn around the coarse yarn by further twisting the fine yarn in said second direction to form a helical, balloon-like spiral wrap that partially opens the twisted structure of the coarse yarn along its length;
plying the coarse yarn and the fine yarn using a Two-For-One (TFO) twisting technique under controlled tension and twist insertion to obtain a plied pile yarn, wherein the plying operation is controlled such that upon fabric formation,
(i) the fine yarn contributes at least two turns per terry loop, and
(ii) the fine yarn migrates towards the base of each of the pile loops to provide a radial confinement and base support while the coarse yarn occupies the loop crown region to maximize an opening volume within the loop structure, thereby producing a plied pile yarn in which the coarse yarn remains structurally bulked and the fine yarn acts as a confinement wrap; and
weaving the plied pile yarn into a terry fabric to form upright profiled pile loops, whereby the terry fabric exhibits enhanced bulk and improved hand feel, and the plied pile yarn exhibits reduced shedding of loose fibers after weaving relative to a comparable terry fabric produced without the opposite-direction fine-yarn wrapping and TFO-controlled loop structure.

5. The method as claimed in claim 4, wherein the warp yarns, weft yarns, coarse yarns, and fine yarns are each independently selected from fibers comprising Organic cotton, BCI cotton, Indian cotton, USA cotton, Supima cotton, Egyptian cotton, Australian cotton, Turkish cotton, naturally colored cotton, naturally dyed cotton, dyed cotton, cotton blended with regenerated or synthetic fibers, cotton/bamboo, cotton/modal, cotton/micro-modal, cotton/tencel, cotton/viscose, cotton/silk, cotton/bamboo/hemp, cotton/hemp, cotton/linen, cotton/ecover, cotton/excel, Egyptian cotton/excel, recycled cotton and its blends, cotton/Naia, cotton/wool, cotton/PVA, cotton/polyester, Regenerative cotton, Kasturi cotton, cotton/PLA, or any combination thereof;

6. The method as claimed in claim 4, wherein the coarse yarn has a yarn count in the range of 6 Ne to 30 Ne and the fine yarn has a yarn count in the range of 20 Ne to 177 Ne.

7. The method as claimed in claim 4, wherein the coarse yarn has a TM in the range of 2.6 to 3.8, and the fine yarn has a TM in the range of 3.0 to 4.8.

8. The method as claimed in claim 4, wherein the controlled plying operation is carried out using the TFO twisting technique to achieve the plied pile yarn with a helical wrap angle in a range from15° to 30°.

9. The method as claimed in claim 4, wherein the plying operation is controlled to achieve a Turns Per Inch (TPI) in a range from2.5 to 13.5 based on a pile height of 2.5 mm to 10 mm.

10. The method of claim 4, wherein the TMs of the coarse yarn and fine yarn are selected to permit partial opening of the coarse yarn under the fine-yarn wrap without collapse of the coarse yarn core during plying.

11. The method of claim 4, wherein the helical spiral wrap of the fine yarn forms a continuous wrap along the coarse yarn with a pitch selected to maintain radial confinement at the loop base region during terry weaving.

12. The method of claim 4, wherein the plying tension applied to the fine yarn is greater than the plying tension applied to the coarse yarn, thereby biasing migration of the fine yarn toward the loop base.

13. The method of claim 4, wherein the plied pile yarn is woven on a terry loom to yield pile loops having a loop height and loop density selected to preserve the partial opening of the coarse yarn crown region.

14. The method as claimed in claim 4, wherein the terry fabric is subjected to a two-sided, to-and-fro tumbling process with optimized tumbling parameters to stabilize loop geometry, enhance bulk and reduce linting.

15. The method as claimed in claim 14, wherein the optimized tumbling parameters comprise:
a speed from 10-13 mpm;
a tumbling time of 5 minutes per tumbling chamber;
a temperature from160-170°C; and
a finishing recipe including silicone and cationic agents including value-added topical finishes.
